



US005880081A

# United States Patent [19]

Gopalkrishnan et al.

[11] Patent Number: **5,880,081**[45] Date of Patent: **Mar. 9, 1999**

[54] **CONCENTRATED BUILT LIQUID DETERGENTS CONTAINING A DYE-TRANSFER INHIBITING ADDITIVE**

5,710,119 1/1998 Busch et al. .... 510/360  
5,723,425 3/1998 Cauwberghs et al. .... 510/299  
5,723,426 3/1998 Zhen et al. .... 510/337

[76] Inventors: **Sridhar Gopalkrishnan**, 8641  
Woodside Dr., Grosse Ile, Mich. 48138;  
**Kathleen M. Guiney**, 423 Maple St.,  
Wyandotte, Mich. 48192

## FOREIGN PATENT DOCUMENTS

0 576 777 A1 1/1994 European Pat. Off. .  
0 576 778 A1 1/1994 European Pat. Off. .  
0 582 478 A2 2/1994 European Pat. Off. .  
0 635 565 A1 1/1995 European Pat. Off. .  
0 635 566 A1 1/1995 European Pat. Off. .  
WO 95/03388 2/1995 European Pat. Off. .  
WO 95/03390 2/1995 European Pat. Off. .  
WO 95/06098 3/1995 European Pat. Off. .  
4027832 3/1992 Germany .

Primary Examiner—Ardith Hertzog  
Attorney, Agent, or Firm—Joanne P. Will

## [57] ABSTRACT

The present invention relates to the formulation of stable, aqueous, concentrated built liquid detergents that contain a dye-transfer inhibiting additive. The invention also relates to a method of incorporating a dye-transfer inhibiting additive to a liquid detergent composition. The invention also relates to a method of stabilizing a liquid detergent composition containing a high molecular weight dye transfer inhibiting additive.

**2 Claims, No Drawings**

## [56] References Cited

### U.S. PATENT DOCUMENTS

|           |        |                   |       |         |
|-----------|--------|-------------------|-------|---------|
| 5,534,183 | 7/1996 | Gopalkrishnan     | ..... | 510/417 |
| 5,536,440 | 7/1996 | Gopalkrishnan     | ..... | 510/434 |
| 5,604,194 | 2/1997 | Cauwberghs et al. | ..... | 510/325 |
| 5,622,926 | 4/1997 | Schade et al.     | ..... | 510/340 |
| 5,627,151 | 5/1997 | Detering et al.   | ..... | 510/475 |
| 5,710,118 | 1/1998 | Busch et al.      | ..... | 510/360 |

**CONCENTRATED BUILT LIQUID  
DETERGENTS CONTAINING A DYE-  
TRANSFER INHIBITING ADDITIVE**

**FIELD OF THE INVENTION**

The present invention relates to the formulation of stable, aqueous, concentrated built liquid detergents that contain a dye-transfer inhibiting additive. The invention also relates to a method of preparing stable liquid detergent compositions containing a dye-transfer inhibiting additive.

**BACKGROUND OF THE INVENTION**

The incorporation of major amounts of builders in liquid detergent compositions poses a significant formulating challenge since the presence of major amounts of builder inevitably causes the detergent composition to phase separate. Builders such as sodium citrate, citric acid, sodium carbonate, and/or alkali metal silicates can only be incorporated in minor amounts in liquid detergent compositions, such amounts being typically below the concentration levels that would cause separation of the surfactant phase. However, the novel hydrophilic copolymers disclosed in U.S. Pat. No. 5,536,440 and U.S. Pat. No. 5,534,183 (both assigned to BASF) are useful in stabilizing concentrated built liquid detergent compositions.

Further, excessive dye-transfer during the washing of garments poses a problem for built liquid detergent formulators. Colored garments which are dyed with dyes having poor fastness, typically release dye during the wash process which then migrate to other garments during the wash thus diminishing the quality and appearance of garments. EP 587550, EP 587549, EP 581753, EP 581752, EP 581751, EP 579295, WO 9402581, WO 9503388, and WO 9506098 disclose the use of polyamine N-oxides as additives for controlling dye transfer during the laundering of garments. EP 576778, EP 576777, EP 582478, EP 635566, EP 635565, WO 9503390, WO 9503388, and WO 9506098 disclose the use of polyvinyl pyrrolidone, polyvinylpyrrolidone-polyvinylimidazole as dye transfer inhibitors for laundry formulations. While there are significant advantages to using polyvinyl pyrrolidone (PVP) as a dye transfer inhibitor, the drawback is that the higher molecular weight polymers of PVP (greater than about 15000 MW) are not stable in liquid laundry formulations. This drawback is particularly problematic for the liquid detergent formulator since the higher molecular weight polyvinyl pyrrolidone polymers have significantly improved dye transfer inhibiting properties. Currently, the art is faced with the problem of how to incorporate high molecular weight polyvinyl pyrrolidone polymers into built liquid laundry formulations without destabilizing the formulation.

The Applicants have discovered that high molecular weight polyvinyl pyrrolidone polymers can now be successfully incorporated into built liquid detergent formulations which contain Applicants' hydrophilic polymer.

**SUMMARY OF THE INVENTION**

The present invention relates to a stable, built liquid detergent composition comprising about 5 to 70% of detergent active matter selected from the group consisting of anionic, nonionic, cationic, amphoteric and zwitterionic surfactants, as well as about 1 to 60% of one or more electrolytes. The detergent composition further comprises 0.1 to 5% of a high molecular weight dye-transfer inhibiting additive. Finally, the liquid detergent composition has about

0.01 to 5% of at least one hydrophilic copolymer comprised of an unsaturated hydrophilic copolymer copolymerized with a hydrophilic oxyalkylated monomer, selected from Formula I, or Formula II, or both, wherein Formula I is:



where x, y, z and a are integers; R3, Q, and M comprise the hydrophilic oxyalkylated monomer sidechain and Q is oxyethylene or a mixture of oxyethylene with C3-C4 oxyalkylene with the proviso that said sidechain has a solubility of at least 500 g/L in water; M is an alkali metal or hydrogen, and said monomer units are in random order; (x+y):z is from 5:1 to 1,000:1, x and y cannot be 0 and y can be zero or equal to any value of x; wherein further, each



and Formula II is:



wherein x, y, z and a are integers; Q, and M comprise the hydrophilic oxyalkylated monomer sidechain and Q is oxyethylene or a mixture of oxyethylene with C3-C4 oxyalkylene with the proviso that said sidechain has a solubility of at least 500 g/L in water; M is an alkali metal or hydrogen, and said monomer units are in random order; (x+y):z is from 5:1 to 1,000:1, x and y cannot be 0 and y can be zero or equal to any value of x; wherein further, each

R<sub>1</sub>=H or CH<sub>3</sub>;

R<sub>2</sub>=COOM, OCH<sub>3</sub>, SO<sub>3</sub>M, O—CO—CH<sub>3</sub>, CO—NH<sub>2</sub>;

The remainder of the detergent formulation is water. The liquid detergent composition has a phase separation of less than about 2% over a one month period.

The invention also relates to a method of stabilizing a liquid detergent composition containing a dye-transfer inhibiting additive which comprises adding thereto about 0.01–5% of at least one hydrophilic copolymer as described hereinabove.

#### DETAILED DESCRIPTION OF THE PREFERRED EMBODIMENT

5

15

The present invention relates to a liquid detergent composition comprising about 5–70% of detergent active matter selected from the group consisting of anionic, nonionic, cationic, amphoteric and zwitterionic surfactants, as well as about 1–60% of one or more electrolytes. The detergent composition further comprises 0.1 to 5% of a high molecular weight dye-transfer inhibiting additive. High molecular weight, as used herein, is defined as a molecular weight of greater than or equal to 15,000. Finally, the liquid detergent composition also has about 0.01–5% of at least one hydrophilic copolymer comprised of an unsaturated hydrophilic copolymer copolymerized with a hydrophilic oxyalkylated monomer, selected from Formula I, or Formula II, or both, wherein Formula I is:



where x, y, z and a are integers; R<sub>3</sub>, Q, and M comprise the hydrophilic oxyalkylated monomer sidechain and Q is oxyethylene or a mixture of oxyethylene with C<sub>3</sub>–C<sub>4</sub> oxyalkylene with the proviso that said sidechain has a solubility of at least 500 g/L in water; M is an alkali metal or hydrogen, and said monomer units are in random order; (x+y):z is from 5:1 to 1,000:1, x and z cannot be 0 and y can be zero or equal to any value of x; wherein further, each

R=H or CH<sub>3</sub>;

R<sub>2</sub>=COOM, OCH<sub>3</sub>, SO<sub>3</sub>M, O—CO—CH<sub>3</sub>, CO—NH<sub>2</sub>;

R<sub>3</sub>=CH<sub>2</sub>—O—, CH<sub>2</sub>—N—, COO—,



and Formula II is:



wherein x, y, z and a are integers; Q, and M comprise the hydrophilic oxyalkylated monomer sidechain and Q is oxyethylene or a mixture of oxyethylene with C<sub>3</sub>–C<sub>4</sub> oxyalkylene with the proviso that said sidechain has a solubility of at least 500 g/L in water; M is an alkali metal or hydrogen, and said monomer units are in random order; (x+y):z is from 5:1 to 1,000:1, x and z cannot be 0 and y can be zero or equal to any value of x; wherein further, each

R<sub>1</sub>=H or CH<sub>3</sub>;

R<sub>2</sub>=COOM, OCH<sub>3</sub>, SO<sub>3</sub>M, O—CO—CH<sub>3</sub>, CO—NH<sub>2</sub>;

The remainder of the detergent formulation is water. The liquid detergent composition has a phase separation of less than about 2% over a one month period.

Also provided as part of the invention is a method of stabilizing a liquid detergent composition containing a dye-transfer inhibiting additive which comprises adding thereto about 0.01–5% of at least one hydrophilic copolymer as described hereinabove.

As heretofore stated, the molar ration of (x+y) to z in both Formulas I and II is within the range of about 5:1 to 1000:1, preferably about 50:1 to 800:1, and more preferably about 100:1 to 200:1. The value of a is within the range of about 1 to 200, more preferably about 1 to 150, and more preferably about 1 to 100.

The total molecular weight of the copolymer will be within the range of about 500 to 500,000, as determined by gel permeation chromatography. It is further desirable that the molecular weight fall within the range of about 1,000 to 100,000, and even more preferably be within the range of about 1,000 to 10,000 WAMW (weight average molecular weight). Molecular weights herein are given in terms of WAMW unless otherwise specified.

The hydrophilic copolymers of the present invention are prepared by copolymerizing two hydrophilic monomers. Specifically, an unsaturated hydrophilic monomer is copolymerized with an oxyalkylated monomer. These monomers may be randomly distributed within the polymer backbone. The Unsaturated Hydrophilic Monomers

The unsaturated hydrophilic monomer may be selected from the group consisting of acrylic acid, maleic acid, 60 maleic anhydride, methacrylic acid, methacrylate esters and substituted methacrylate esters, vinyl acetate, as well as vinyl acetate copolymerized with said oxyethylated monomer and hydrolyzed to polyvinyl alcohol, methylvinyl ether, and vinylsulphonate. Preferably, the unsaturated hydrophilic 65 monomer component of the hydrophilic copolymer is acrylic acid. Other useful monomers will include crotonic acid, itaconic acid, as well as vinyl acetic acid.

### The Oxyalkylated Monomers

Examples of the oxyalkylated monomers include compounds that have a polymerizable olefinic moiety with at least one acidic hydrogen and are capable of undergoing addition reaction with alkylene oxide. Also included are monomers with at least one acidic hydrogen that are polymerized first, and then subsequently oxyalkylated to yield the desired product. For example, allyl alcohol is especially preferred since it represents a monofunctional initiator with a polymerizable olefinic moiety having an acidic hydrogen on the oxygen, and is capable of adding to alkylene oxide. Similarly, diallyamine represents another monofunctional initiator with polymerizable olefinic moieties, having an acidic hydrogen on the nitrogen, and is capable of adding to alkylene oxide. Other examples of the oxyalkylated monomer of the copolymer will include reaction products of either acrylic acid, methacrylic acid, maleic acid, or 3-allyloxy-1,2-propanediol with alkylene oxide.

The molecular weight of the oxyalkylated monomer in Formula I or II, according to the various embodiments of the invention will be within the range of about 200 to 30,000, more preferably about 500 to 15,000, and even more preferably about 1,000 to 5,000.

The oxyalkylated moiety represents the side chain of this monomer. The side chain is hydrophilic in nature, that is, the side chain when isolated from its linkage to the backbone carbon atom is completely soluble in water. The monomer unit containing the hydrophilic side chain also has similar solubility characteristics as the side chain. Preferably, the side chain when isolated from its linkage to the backbone will have a solubility in water of at least about 700 grams/liter, and even more preferably about 1000 grams/liter, or more. Moreover, the entire side chain is hydrophilic in nature by virtue of its extensive solubility in water.

### Preparation of the Hydrophilic Copolymers Useful in the Practice of the Present Invention

The hydrophilic copolymers of the present invention are prepared by copolymerizing two hydrophilic monomers. Specifically, an unsaturated hydrophilic monomer is copolymerized with an oxyalkylated monomer. These monomers may be randomly distributed within the polymer backbone. The method of preparation of these hydrophilic copolymers is described in U.S. Pat. No. 5,536,440 and U.S. Pat. No. 5,534,183, incorporated by reference herein. Further, the following non-limiting example illustrates the preparation of the hydrophilic copolymers useful in the practice of the present invention.

### Preparation of Ethylene Oxide Adduct of Allyl Alcohol (I)

To a 1 gallon stainless steel autoclave equipped with steam heat, vacuum and nitrogen pressure capability and agitation, a homogenous mixture of 210.5 grams of allyl alcohol and 23.4 grams of potassium +butoxide was charged. The vessel was sealed, purged with nitrogen and pressurized to 90 psig 80° C. The first 75 grams of ethylene oxide was charged over a 1 hour period at 75° to 85° C. and <90 psig pressure. The next 125 grams of ethylene oxide was charged over a 1 hour period at 75°-85° C. and <90 psig. The next 225 grams of ethylene oxide was charged over a 1 hour period at 100°-110° C. and <90 psig. The remaining 2140.9 grams of ethylene oxide was added over an 8 hour period at 145°-155° C. and <90 psig pressure. After all of the ethylene oxide was added, the mixture was reacted at 150° C. for 2 hours and the vessel was vented to 0 psig. The material was stripped at <10 mm Hg and 125° C. for 1 hour then cooled to 50° C. and discharged into an intermediate holding tank for analysis.

To a 2 gallon stainless steel autoclave equipped with steam heat, vacuum, nitrogen pressure capability and

agitation, 498.8 grams of the allyl alcohol ethylene oxide intermediate was charged. The vessel was sealed and pressurized to 90 psig with nitrogen and vented to 2 psig. This was repeated two more times. The temperature was adjusted to 145° C. and the pressure was readjusted to 34 psig with nitrogen. To the vessel, 2198.3 grams of ethylene oxide was charged at 275 grams per hour. The temperature was maintained at 140°-150° C. and the pressure was maintained at <90 psig. If the pressure rose above 85 psig, the ethylene oxide addition was slowed. If this failed to lower the pressure, the addition was halted and allowed to react at 145° C. for 30 minutes. The vessel was slowly vented to a 0 psig and repadded to 34 psig with nitrogen. The addition was continued at 140° to 150° C. and <90 psig pressure. After all of the ethylene oxide was added, the material was held at 145° C. for 1 hour. It was then cooled to 90° C. and 2.9 grams of 85% phosphoric acid was added. The material was mixed for 30 minutes and then vacuum stripped at 100° C. for 1 hour. The batch was cooled to 70° C. and discharged into a holding tank. The product was found to have a number average molecular weight of 4095 g/mol by phthalic anhydride esterification in pyridine.

### Copolymerization of (I) with Acrylic Acid

To a two liter, four-necked flask equipped with a mechanical stirrer, reflux condenser, thermometer, and outlet for feed lines, were added 301 grams of distilled water and 2.6 grams of 70% phosphorous acid. This solution was heated to 95° C. at which time a monomer blend of 555.4 grams of glacial acrylic acid and 62.8 grams of an allyl alcohol initiated ethoxylate (molecular weight @ 3800), a redox initiator system consisting of 132 grams of a 38% sodium bisulfate solution and 155.2 grams of a 10.9% sodium persulfate solution, are fed into the flask linearly and separately while maintaining the temperature at 95° (+/-3) C. The sodium bisulfate solution and monomer blend feeds are added over 4 hours while the sodium persulfate solution is added over 4.25 hours. The three feeds are added via TEFILON® 1/8 inch tubing lines connected to rotating piston pumps. Appropriately sized glass reservoirs attached to the pumps hold the monomer blend and initiator feeds on balances accurate to 0.1 gram to precisely maintain feed rates. When the additions are complete, the system is cooled to 80° C. At this temperature, 25.3 grams of a 2.4% 2,2'-Azobis (N,N'-dimethyleneisobutylramidine) dihydrochloride solution is added to the system over 0.5 hours as a postpolymerizer. When addition is complete the system is reacted for 2 hours at 80° C. After reaction, the system is cooled to 60° C. and the solution pH is adjusted to about 7 with the addition of 658 grams of 50% sodium hydroxide solution. The resultant neutral polymer solution has an approximate solids content of about 40%.

### Preparation of the Detergent Composition of the Present Invention

The hydrophilic copolymer prepared as described hereinbefore is added to detergent compositions, to impart stability thereto. See U.S. Pat. No. 5,536,440 and U.S. Pat. No. 5,534,183 incorporated by reference herein. Stable detergent compositions are those that do not give more than about a 2% phase separation upon storage at room temperature for a period of one month (30) days from the time of preparation. Preferably, the phase separation is within the range of about 0-2%, and even more preferably less than about 1 %. The volume fraction of the separated aqueous phase is measured as a function of the total volume of the sample. For example, if the total volume of the sample is 100 mL, then a 2% separation would correspond to 2 mL.

The hydrophilic copolymer will therefore comprise about 0.01 to 5% by weight of the liquid detergent composition.

Preferably, the hydrophilic copolymer of the invention will make up about 0.5 to 4% of a typical laundry formulation, even more preferably about 1 to 2%. (Unless otherwise stated, all weight percentages are based upon the weight of the total laundry formulation).

The laundry formulation will preferably contain about 5 to 70% of detergent active matter, more preferably about 15 to 40%, and most preferably about 25 to 35%.

Said detergent active matter may be selected from the group of anionic, nonionic, cationic, amphoteric and zwitterionic surfactants known to the skilled artisan. Examples of these surfactants may be found to McCutcheon, *Detergents and Emulsifiers* 1993, incorporated herein by reference. Examples of nonionic surfactants will include commonly utilized nonionic surfactants which are either linear or branched and have an HLB of from about 6 to 18, preferably from about 10 to 14. Examples of such nonionic detergents are 30 alkylphenol oxyalkylates (preferably oxyethylates) and alcohol oxyethylates. Examples of the alkylphenol oxyalkylates include C<sub>6</sub>–C<sub>18</sub> alkylphenols with about 1–15 moles of ethylene oxide or propylene oxide or mixtures of both. Examples of alcohol oxyalkylates include C<sub>6</sub>–C<sub>18</sub> alcohols with about 1–15 moles of ethylene oxide or propylene oxide or mixtures of both. Some of these types of nonionic surfactants are available from BASF Corp. under the trademark PLURAFAC. Other types of nonionic surfactants are available from Shell under the trademark NEODOL. In particular, a C<sub>12</sub>–C<sub>15</sub> alcohol with an average of 7 moles of ethylene oxide under the trademark NEODOL® 25-7 is especially useful in preparing the laundry detergent compositions useful in the invention. Other examples of nonionic surfactants include products made by condensation of ethylene oxide and propylene oxide with ethylene diamine (BASF, TETRONIC® and TETRONIC® R). Also included are condensation products of ethylene oxide and propylene oxide with ethylene glycol and propylene glycol (BASF, PLURONIC® and PLURONIC® R). Other nonionic surface active agents also include alkylpolyglycosides, long chain aliphatic tertiary amine oxides and phosphine oxides.

Typical anionic surfactants used in the detergency art include the synthetically derived water-soluble alkali metal salts of organic sulphates and sulphonates having about 6 to 22 carbon atoms. The commonly used anionic surfactants are sodium alkylbenzene sulphonates, sodium alkylsulphates and sodium alkylether sulphates. Other examples include reaction products of fatty acids with isethionic acid and neutralized with sodium hydroxide, sulphate esters of higher alcohols derived from tallow or coconut oil, and alpha-methylestersulfonates.

Examples of amphoteric detergents include straight or branched aliphatic derivatives of heterocyclic secondary or tertiary amines. The aliphatic portion of the molecule typically contains about 8 to 20 carbon atoms. Zwitterionic detergents include derivatives of straight or branched aliphatic quaternary ammonium, phosphonium or sulphonium compounds.

Further, the laundry detergent formulation will also contain one or more electrolytes. Electrolytes defined herein are any ionic water-soluble material. The presence of the electrolyte is often required to bring about the structuring of the detergent active material, although lamellar dispersions are reported to be formed with detergent active material alone in the absence of a suitable electrolyte. Electrolytes typically comprise from about 1 to 60% by weight, and more preferably about 10 to 45% by weight and, most preferably about 25 to 35% of a laundry detergent formulation.

Examples of suitable electrolytes include compounds capable of providing sufficient ionic strength to the aqueous detergent composition. These compounds would include alkali metal salts of citric acid, alkali metal carbonates, and alkali metal hydroxides. Of these, sodium citrate, sodium carbonate and sodium hydroxide are preferred. Potassium salts can also be incorporated to promote better solubility. Other examples of suitable electrolytes will include the phosphate salts such as sodium or potassium tripolyphosphate, and alkali metal silicates.

In many cases the electrolyte utilized will also serve as the builder for enhancing detergency. The builder material sequesters the free calcium or magnesium ions in water and promote better detergency. Additional benefits provided by the builder are increased alkalinity and soil suspending properties. With the near phase-out of phosphate in household laundry detergents, the most commonly used non-phosphate builders are the alkali metal citrates, carbonates, bicarbonates and silicates. All of these compounds are water-soluble. Water-insoluble builders which remove hardness ions from water by ion-exchange mechanism are the crystalline or amorphous aluminosilicates referred to as zeolites. Mixtures of electrolytes or builders can also be employed. Generally, the amount of electrolyte used in laundry detergent compositions according to the invention will be will above the solubility limit of the electrolyte. Thus, it is possible to have undissolved electrolyte which remains suspended in the liquid matrix. Secondary builders such as the alkali metals of ethylene diamine tetraacetic acid, nitrilotriacetic acid can also be utilized in the laundry formulations of the invention. Other secondary builders known to those skilled in the art may also be utilized.

The laundry detergent formulations heretofore described may also contain additional ingredients such as enzymes, anti-redeposition agents, optical brighteners, as well as dyes and perfumes known to those skilled in the art. Other optional ingredients may include fabric softeners, foam suppressants, and oxygen or chlorine releasing bleaching agents.

Finally, the laundry detergent compositions will also contain a high molecular weight dye-transfer inhibiting additive. Commonly used dye-transfer inhibiting additives are polyvinyl pyrrolidone, copolymers of vinylpyrrolidone with vinylimidazole, polyamine N-oxides. Preferably the dye transfer inhibiting additive is polyvinyl pyrrolidone (PVP). Preferably, the dye transfer inhibiting additive is polyvinyl pyrrolidone with a molecular weight of 15,000 to 500,000, more preferably 20,000 to 100,000, most preferably about 40,000 molecular weight. Said dye transfer inhibiting additive is present at a level of 0.1 to 5.0%, more preferably at a level of 0.3 to 4% and most preferably at a level of 0.5 to 2%. High molecular weight, as used herein, is defined as a molecular weight of greater than or equal to 15,000.

## EXAMPLES

The following examples will serve to demonstrate the stability of the liquid detergent compositions containing high molecular weight dye transfer inhibiting additives, according to various embodiments of the invention. These examples should not be construed as limiting the scope of the invention.

The examples describe the aqueous liquid detergent compositions of this invention which are stable. The numbers in each column refer to the active weight percentage of each component in the detergent formulation. The stability of the dye-transfer additive (PVP molecular weight 40,000) was

first investigated in commercially available liquid detergents. The results from these tests are shown in Example-1. In each commercial liquid detergent, physical instability was observed 24 hours after preparation, when the dye transfer inhibiting additive was added to the liquid detergent.

| Example 1                   |                              |                            |
|-----------------------------|------------------------------|----------------------------|
| Commercial Liquid Detergent | % Polyvinylpyrrolidone (PVP) | Stability                  |
| Tide ®                      | 2%                           | Unstable; Phase Separation |
| All ®                       | 2%                           | Unstable; Phase Separation |
| Wisk ®                      | 2%                           | Unstable; Phase Separation |
| Fab ®                       | 2%                           | Unstable; Phase Separation |
| Purex ®                     | 2%                           | Unstable; Phase Separation |

Example-2 shows a stable, concentrated built liquid detergent composition containing a significant amount of a polyvinyl pyrrolidone having a molecular weight of 40,000 and the hydrophilic copolymer as described hereinbefore. This detergent formulation was stable when stored at 25° C. for over two months and also showed excellent stability with 0% phase separation, when stored at 45° C. for over a month.

| Example 2                        |          |
|----------------------------------|----------|
| Ingredient                       | % Active |
| Sodium LAS                       | 22       |
| Nonionic surfactant              | 7        |
| Sodium Citrate Dihydrate         | 5        |
| Sodium Carbonate                 | 8        |
| Zeolite A                        | 10       |
| Sokalan ® HP53 polymer           | 2        |
| Hydrophilic Polymer of Formula I | 1        |
| Water                            | Balance  |
| Viscosity                        | 522cps   |
| Stability                        | STABLE   |

The nonionic surfactant used in the formulations shown in the Tables is NEODOL® 25-7, a product of Shell. The linear alkylbenzene sulfonic acid, sodium salt (LAS) was obtained from Vista under the name Vista C-560 slurry. The zeolite (builder) was "ZEOLITE A", also known as VALFOR® 100, available from the PQ Corporation of Valley Forge, Pa. Sodium carbonate (builder) was obtained from the FMC Corporation under the name FMC. Grade 100. The sodium citrate dihydrate (builder) was obtained from Haaman & Reimer. Unless otherwise indicated, the hydrophilic polymer used in the formulations was a copolymer of acrylic acid with an oxyethylated allyl alcohol. The ratio of acrylic acid to oxyethylated allyl alcohol was about 93:7 by weight, while the molar ratio was about 116:1. The molecular weight of the oxyethylated monomer was about 700. R<sub>1</sub>=HR<sub>2</sub>=COOM, R<sub>3</sub>=CH<sub>2</sub>—O, and y=O. The Sokalan® HP53 polymer (dye transfer inhibiting additive) used is polyvinyl pyrrolidone with a molecular weight of 40,000. SOKALAN® is a registered trademark of the BASF Corporation.

We claim:

1. A method of stabilizing a liquid detergent composition containing a high molecular weight dye transfer inhibiting additive, said dye transfer inhibiting additive having a molecular weight of greater than or equal to 15,000, selected from the group consisting of polyvinylpyrrolidone, vinylpyrrolidone -vinylimidazole copolymers, polyamine N-oxides, and mixtures thereof; comprising adding to said

composition 0.01 to 5% by weight of at least one hydrophilic copolymer comprised of an unsaturated hydrophilic copolymer, copolymerized with a hydrophilic oxyalkylated monomer, wherein said hydrophilic copolymer is Formula I, or Formula II, or both:



where x, y, z and a are integers; R<sub>3</sub>, Q, and M comprise the hydrophilic oxyalkylated monomer sidechain and Q is oxyethylene or a mixture of oxyethylene with C<sub>3</sub>—C<sub>4</sub> oxyalkylene with the proviso that said sidechain has a solubility of at least 500 g/L in water; M is an alkali metal or hydrogen, and the monomer units are in random order; (x+y):z is from 5:1 to 1,000:1, x and z cannot be 0 and y can be zero or equal to any value of x; wherein further, each

R=H or CH<sub>3</sub>;  
R<sub>2</sub>=COOM, OCH<sub>3</sub>, SO<sub>3</sub>M, O—CO—CH<sub>3</sub>, CO—NH<sub>2</sub>;  
R<sub>3</sub>=CH<sub>2</sub>—O—, CH<sub>2</sub>—N—, COO—, —O—,



and Formula II is:



wherein x, y, z and a are integers; Q, and M comprise the hydrophilic oxyalkylated monomer sidechain and Q is oxyethylene or a mixture of oxyethylene with C<sub>3</sub>—C<sub>4</sub> oxyalkylene with the proviso that said sidechain has a solubility of at least 500 g/L in water; M is an alkali metal or hydrogen, and said monomer units are in random order; (x+y):z is from 5:1 to 1,000:1, x and z cannot be 0 and y can be zero or equal to any value of x; wherein further, each

R<sub>1</sub>=H or CH<sub>3</sub>;  
R<sub>2</sub>=COOM, OCH<sub>3</sub>, SO<sub>3</sub>M, O—CO—CH<sub>3</sub>, CO—NH<sub>2</sub>.  
2. A method according to claim 1, wherein in Formula I, R<sub>1</sub>=H, R<sub>2</sub>=COOM, R<sub>3</sub>=—CH<sub>2</sub>—O; Q is oxyethylene; y=O.

\* \* \* \* \*